

## 1

2,706,677

## AMINES AND AMIDES AS ANTI-STALLING ADDITIVES

Gordon W. Duncan, Westfield, William E. Lifson, Elizabeth, and Joseph P. Haworth, Westfield, N. J., assignors to Esso Research and Engineering Company, a corporation of Delaware

No Drawing. Application June 28, 1950,  
Serial No. 170,944

4 Claims. (Cl. 44—71)

The present invention relates to a motor fuel composition adapted to provide distinct improved motor operation under cool moist operating conditions. The motor fuel composition of the present invention comprises a hydrocarbon mixture boiling in the gasoline boiling range which contains as an ingredient a very small percentage of a high boiling amine. In addition, the fuel compositions of the present invention may contain solvent oil and other additives such as lead alkyl anti-detonants, dyes, gum inhibitors, oxidation inhibitors, and the like.

The novel fuel compositions of this invention are primarily intended to overcome certain operational difficulties in connection with automotive, marine, stationary, and airplane engines. The difficulties referred to result in frequent stalling of the engine under idling conditions. This stalling may be encountered whenever the weather conditions in which the engine is used are such as to provide a relatively high humidity, and a temperature below about 60° F.

While this problem has actually been existent for many years, attention has recently been focused on it due to numerous complaints of car owners particularly in the northern portion of the United States. These owners report that during cool, wet weather their cars give poor idling performance characterized by a high number of engine stalls. The difficulty is encountered in all types of cars employing all types of carburetors and utilizing all commercial brands of gasoline.

In order to indicate the magnitude of this difficulty, reference may be made to a survey conducted in the New Jersey area based on the experiences of 300 car owners driving twenty different car models, during the fall and winter period. These cars employed the winter grade of regular and premium commercial gasolines. Table I gives a summary of the results obtained, showing the substantial number of stalls encountered in the operation of the cars under the indicated conditions.

TABLE I

|                             | Number of Complaints of Two Stalls or More<br>(Per 100 Cars) |          |            |            |      |
|-----------------------------|--------------------------------------------------------------|----------|------------|------------|------|
| Temperature, ° F.           | 32                                                           | 35       | 37         | 52         | 56   |
| Relative Humidity, Percent. | 52                                                           | 70       | 96         | 100        | 96   |
| Weather                     | Clear                                                        | Overcast | Light Rain | Heavy Rain | Rain |
| Winter Regular Users        | 5                                                            | 15       | 20         | 21         | 7    |
| Winter Premium Users        | 6                                                            | 38       | 40         | 42         | 2    |

The bare statistics of Table I coupled with the common experience of all automotive users serves to indicate the magnitude of the problem of engine stalling encountered under cool, humid temperature conditions. However, it is significant to note that this problem has of late become of increased importance due to certain specific factors. First, most postwar cars are now provided without a manual throttle so that car owners are no longer able to increase the idle speed during the warm-up period to prevent stalling. Second, the idle speed of cars with automatic transmissions is rather critical during a warm-up and the fastest idle which may be used must not be too fast, increasing the criticality of stalling conditions. Third, stalling of a car with automatic transmission frequently does not occur until the driver is ready to accel-

erate, so that just at this most inconvenient time it is necessary to shift the car to neutral, restart the engine, and shift back into gear; magnifying the inconvenience of frequent stalls. A fourth factor affecting the magnitude of stalling difficulties relates to the volatility of the fuels now provided for automotive use. The volatility of commercial fuels over a period of years has been increased sufficiently to increase stalling difficulties as will be brought out herein.

On investigating this problem, it has been determined that the cause of repeated engine stalling in cool, humid weather is the formation of ice in the carburetor of the engine. On a cool, moist day, gasoline evaporating in the carburetor exerts sufficient refrigerating effect to condense and freeze moisture present in the air entering the carburetor. Normal fuel vaporization within the carburetor can cause a temperature reduction of the metal parts of the carburetor up to 50° F. below that of the entering air. Consequently, prior to the time of complete engine and radiator warm-up, this drop in temperature may cause formation of ice in the carburetor. Ice formation probably occurs most readily under conditions of light load operation. The result is that after a period of light load operation, when the throttle is closed to the idle position, ice already formed on the throttle plate and adjacent walls, plus ice which then forms, restricts the narrow air openings to cause engine stalling.

To more clearly define the problem of engine stalling due to carburetor icing, data were tabulated based on customer reaction surveys, carefully controlled road tests, and laboratory cold room engine performance tests. These tests show that carburetor icing depends primarily upon atmospheric temperature and humidity conditions. The tests show that stalling difficulties due to ice formation in the carburetor are not encountered below about 30° F., nor above about 60° F. when employing fuels having conventional volatility characteristics. Similarly, these tests demonstrate that stalling is only encountered when the humidity is in excess of about 65%.

Another factor having a bearing on the formation of ice in the carburetor, is the volatility of the fuel employed. To determine this effect laboratory cold room tests were conducted to evaluate the stalling characteristics during warm-up of a number of fuels varying in volatility. In these tests a 1947 Chrysler car was installed in a room equipped with temperature and humidity controls. While the temperature and humidity were maintained at particular levels, the stalling characteristics of the car were determined during the warm-up period. The procedure employed was to start the car and to then immediately raise the engine speed to 1500 R. P. M. This speed was maintained for 30 seconds, after which the engine was allowed to idle for 15 seconds. If the engine stalled before 15 seconds had expired, the car was again started and raised to a speed of 1500 R. P. M. for 30 seconds, while if stalling did not occur, the speed was immediately increased to 1500 R. P. M. after the 15 second idling time. The alternate cycles of 30 seconds at 1500 R. P. M. followed by 15 seconds at idling were repeated until the engine was completely warmed up. The number of stalls encountered during this procedure, and up to the time of complete engine warm-up were then recorded. Tests were conducted at 40° F. and at a relative humidity of 100% employing three fuels of varying volatilities. The most volatile fuel was a premium grade of commercial gasoline having a 10% ASTM distillation point of 110° F., a 50% point of 190° F., and a 90% point of 294° F. It was found that this fuel resulted in about 14 or 15 stalls during warm-up. A medium volatility fuel was also tested, consisting of a regular grade commercial gasoline having ASTM distillation characteristics such that 10% distilled at 121° F., 50% distilled at 220° F. and 90% distilled at 342° F. The number of stalls encountered with this fuel were 11. Finally a low volatility gasoline was subjected to the same test procedure. The gasoline had ASTM distillation 10, 50, and 90% points, at 126° F., 270° F. and 387° F. It was found that 5 stalls were encountered with this fuel.

As indicated by these data, carburetor icing is related to the volatility of the fuel employed. Thus, the least volatile fuel tested above, having a 50% distillation point

of 270°, only resulted in 5 stalls, while the highest volatility fuel, having a 50% distillation point of 190° F., resulted in 15 stalls. Extrapolating these data as to the volatility of the fuel, it appears that a fuel having a volatility such that the ASTM 50% distillation point is 310° F., or higher would not be subject to stalling difficulties during warm-up. It must be appreciated, however, that a fuel having ASTM distillation characteristics of this nature would not be desirable as regards warm-up time, cold engine acceleration, economy and crank case dilution. However, in appreciating the scope of the present invention, it is important to note that this invention is only of application to gasoline fuels having an ASTM 50% distillation point below about 310° F. At the same time, as will be brought out, it is possible to correlate the quantity of additives required to overcome icing problems with the volatility of the fuel to be improved. In other words, smaller proportions of additives may be employed with fuels of relatively low volatility, while higher proportions of additives may be required with fuels of higher volatility. Also, it should be appreciated that even when complete stalling does not occur there may be a marked loss of power output due to icing. This is particularly serious in the case of aviation engines. For example, 30% of the light plane mishaps occurring in the United States in 1947 and 1948 were attributed to the formation of ice in the carburetor or intake manifold, which reduced power output by restricting the flow of combustible mixture to the cylinders.

It has now been discovered that distinct operating advantages are secured with respect to stalling, providing a relatively small critical amount of a high boiling amine is utilized. It is preferred that the high boiling amine contain from about 3 to 18 carbon atoms in the molecule. Primary amines are selected from the class of amines represented by the formula  $RNH_2$ , wherein R represents an alkyl group having from 8 to 18 carbon atoms in the molecule. Suitable amines of this class are, for example, cocamine ( $C_8$  to  $C_{18}$  amine), lauryl amine, nonyl amine, and other high boiling alkyl amines.

Secondary amines are selected from the class of compounds represented by the formula  $R_1R_2NH$ , wherein  $R_1$  and  $R_2$  represents hydrocarbon radicals containing from 8 to 18 carbon atoms in the molecule. Suitable amines of this class are, for example, dinormal butyl amine, di-isobutyl amine, and the like.

Suitable tertiary amines are, for example, trinormal butyl amine, tri-isobutyl amine, dialkyl formamide such as dimethyl formamide and diethyl formamide, di-ethyl acetamide as well as di-ethyl amino ethanol are satisfactory. These compounds may be represented by the formula  $R_1R_2NR_3$ , wherein  $R_1$  and  $R_2$  represent hydrocarbon radicals and  $R_3$  represents a hydrocarbon radical or an acyl alkanol radical.

The amount of high boiling amine employed should be appreciably less than about 1% by volume based upon the volume of gasoline present. A concentration of dimethyl formamide within the range from about 0.2% to 0.5% by volume, and especially about 0.25% by volume, is markedly effective.

The present invention may be more fully understood by the following example illustrating the same:

#### EXAMPLE

5 A Continental light aircraft engine was operated on an aviation grade fuel, and on a blend of the fuel and 0.5 volume per cent of various amines. The base fuel had the following distillation characteristics:

10 Engler distillation—

|                               |        |     |
|-------------------------------|--------|-----|
| Initial                       | ° F... | 100 |
| 50%                           | ° F... | 200 |
| Final                         | ° F... | 325 |
| Reid vapor pressure, p. s. i. |        | 7   |

15 The intake air had a temperature of 50° F. and a relative humidity of  $97 \pm 3\%$ . The temperature of the air surrounding the carburetor was 50° F. The throttle was fixed to give an initial engine speed of 1750 R. P. M. and the loss in speed after operation for 3 minutes and 20 for 10 minutes was determined. The results secured are as follows:

#### Carburetor icing in Continental engine anti-icing additive effectiveness

25 [Initial engine speed (fixed throttle), 1750 R. P. M.; intake air, 50° F.,  $97 \pm 3\%$  relative humidity; air surrounding carburetor, 50° F.]  
(Amount of carburetor ice accumulated is reflected in magnitude of speed loss)

| 30 | Additive           | Concentration in Fuel, Vol. Percent | Loss in Speed Due to Icing After 3 Minutes, R. P. M. |
|----|--------------------|-------------------------------------|------------------------------------------------------|
| 35 | None               |                                     | 425                                                  |
|    | Dimethyl Formamide | .25                                 | 0                                                    |
|    | Cocoanut Amine     | 0.10                                | 95                                                   |

40 From the above it is apparent that high boiling amines, particularly dimethyl formamide is very effective.

Having described the invention, it is claimed:

1. A composition comprising a mixture of hydrocarbons boiling in the gasoline boiling range containing from about .2 to .5% by volume of dimethyl formamide.
- 45 2. Composition as defined by claim 1 wherein said composition comprises an aviation motor fuel.
3. A composition comprising a mixture of hydrocarbons boiling in the gasoline boiling range containing about 0.25% by volume of dimethyl formamide.
- 50 4. Composition as defined by claim 3 wherein said composition comprises an aviation motor fuel.

#### References Cited in the file of this patent

#### UNITED STATES PATENTS

|    |           |                |               |
|----|-----------|----------------|---------------|
| 55 | 1,940,445 | Calcott et al. | Dec. 19, 1933 |
|    | 1,947,219 | Murrill        | Feb. 13, 1934 |
|    | 1,992,014 | Rogers et al.  | Feb. 19, 1935 |
| 60 | 2,230,844 | Miller et al.  | Feb. 4, 1941  |
|    | 2,324,118 | Sweeney        | July 13, 1943 |